

July 1, 1930.

W. M. CHACE

1,769,623

THERMOSTATIC ELEMENT

Filed Aug. 16, 1928



MOVEMENT IN INCHES

INVENTOR.  
WILLIAM M. CHACE

BY

Charles E. Hinman  
ATTORNEY.

## UNITED STATES PATENT OFFICE

WILLIAM M. CHACE, OF DETROIT, MICHIGAN; ADELBERT H. LINDLEY, ARTHUR COOPER, AND HILMA B. CHACE, EXECUTORS OF SAID WILLIAM M. CHACE, DECEASED, ASSIGNEES TO W. M. CHACE VALVE COMPANY, OF DETROIT, MICHIGAN, A CORPORATION OF MICHIGAN

## THERMOSTATIC ELEMENT

Application filed August 16, 1928. Serial No. 299,957.

This invention relates to bimetallic elements consisting of two metal strips of dissimilar thermal characteristics and ordinarily used in the control of operation of various instrumentalities, and the purpose of the invention is to provide a bimetallic element capable of being subjected to fairly high heat without permanent deformation.

A further object of the invention is to provide a bimetallic element in which the dissimilar characteristics are not materially apparent below 350 degrees F., or about 550 degrees F., within which temperature range the dissimilar thermal characteristics are most pronounced.

A bimetallic element of such specific character having such a short range of difference in degree of expansion per degree of temperature change is very rapid in its action within the said temperature range and if for instance used in the making or breaking of an electric circuit permits a ready adjustment of parts to insure the making or breaking of the circuit, or other function depending upon the apparatus controlled, at a predetermined temperature.

A further feature of the invention is in the composition of elements permitting the same to be rolled in the usual manner while hot without the production of scale and subsequently finished to the desired thinness while cold. Thus, in view of the absence of pitted surface, very smooth polished surface is produced and a subsequent operation such as grinding or polishing is avoided.

In attaining of these various objects I form the bimetallic element of two metals of dissimilar thermal characteristics both of which contain nickel. While it is well known to utilize nickel in both elements of a thermostatic couple, it has been usual to utilize a fairly high percentage of copper in the expansion side but I have discovered a composition for the expansion side in which the nickel and copper content is small and having a coefficient of expansion approximately equal to that of brass. This invention is more particularly directed to a composition of metals for the expansion side in the provision of a bimetallic element having

the characteristics stated. Preferably, however, what may be termed the neutral or non-expansive side is formed of the following composition—

|         |       |    |
|---------|-------|----|
| Carbon  | 35    | 55 |
| Silicon | 2.00  |    |
| Nickel  | 40.00 |    |
| Iron    | 57.65 |    |

For the expansion side I use the following composition of elements substantially within the range of percentages stated—namely,

|              |                |    |
|--------------|----------------|----|
| Carbon       | .25 to .35     | 65 |
| Silicon      | 1.75 to 2.00   |    |
| Chromium     | 13.25 to 14.00 |    |
| Nickel       | 7.25 to 7.75   |    |
| Copper       | 2.00 to 4.00   |    |
| Wrought iron | 72.50 to 71.90 | 70 |

The elements stated are the usual commercial form and the iron utilized in the expansion side is preferably what is known as "Sweedish iron" particularly in view of its containing a trace of copper and therefore more readily combined with the copper.

In combining these elements I have discovered a method (which is the subject matter of another application for Letters Patent of the United States) whereby the copper is readily mixed with the iron with which it does not readily assimilate. This method consists in the combining of the copper and the nickel between which there is an affinity and then combining the nickel-copper combination with the iron and other ingredients which is readily accomplished due to the affinity between the nickel and iron.

A bimetallic element formed of the two composite metals welded together has the characteristic of temperature change as shown in the accompanying diagram in which the horizontal lines indicating the temperature and the heavy line with the curve showing the deformation of the thermostatic couple under temperature change. From this diagram it will be observed that at temperatures approximately up to 350 degrees F., there is very little movement occasioned, or in other words—the dissimilar thermal charac-

teristics are not pronounced, but from 350 to 500 degrees F., the movement is rapid. That is within this temperature range the dissimilar thermal characteristics are very pronounced and, at temperatures above 550 degrees F., either the expansion is similar or the metals have practically reached their limit of expansion.

In the formation of the bimetallic element two sheets or bars of the respective compositions are welded together a flux being used between the contacting surfaces. The bars or sheets are then rolled while hot to nearly the thinness desired in the final structure and, by reason of the composition utilized on the expansion side, there is no formation of scale in this rolling process which is productive of a pitted surface. Therefore, the stock may be rolled cold to the final thinness thereby producing a practically smooth finished surface as it comes from the rolls. Consequently a final polishing operation is avoided.

One of the purposes of the invention is to provide a bimetallic element that has little movement outside a specific temperature range of about 200 degrees F., as is indicated by the movement curve of the diagram. This diagram is platted from the behavior of a strip of metal .048 inch thick by one-half inch wide and 5½ inches long held stationary at one end free to move at the opposite end.

It will thus be seen that I have secured a bimetallic element in which the greatest difference in degree of expansion per degree of temperature change is within a range of approximately 200 degrees F., and in which the movement is very rapid. This is of value in that it enables the structure with which my improved bimetallic element is to be utilized to be readily set to operate at a specific temperature within the said temperature range.

In bimetallic elements in which the dissimilar thermal characteristics are practically constant up to a point where permanent deformation takes place, it is a very difficult matter to provide mechanical structures that would operate at predetermined temperature as the movement of the element is not restricted to any specific temperature range and an ideal bimetallic element for operation at a specific temperature would be one in which the movement was confined to just that temperature. This, of course, is impossible so far as I now know but I believe that in the provision of such an element in which the pronounced movement is practically confined to a range of approximately 200 degrees F., is a closer approach to the ideal condition than has heretofore been attained.

I have also found that by use of the composition stated I have secured a bimetallic element that may be subjected to temperatures as high as 2000 degrees F., without permanent deformation.

Having thus briefly described my inven-

tion, what I claim and desire to secure by Letters Patent of the United States is—

1. A bimetallic thermostat consisting of two metal parts welded together, one of said parts consisting of the following elements approximately of the stated percentage—

|         |       |       |
|---------|-------|-------|
| Carbon  | ----- | .35   |
| Silicon | ----- | 2.00  |
| Nickel  | ----- | 40.00 |
| Iron    | ----- | 57.65 |

and the other part consisting of the following elements approximately of the percentage stated—viz:

|              |       |                |
|--------------|-------|----------------|
| Carbon       | ----- | .25 to .35     |
| Silicon      | ----- | 1.75 to 2.00   |
| Chromium     | ----- | 13.25 to 14.00 |
| Nickel       | ----- | 7.25 to 7.75   |
| Copper       | ----- | 2.00 to 4.00   |
| Wrought iron | ----- | 72.50 to 71.90 |

2. A bimetallic thermostat consisting of two metal parts welded together each containing nickel and having dissimilar thermal characteristics, the part having the lower coefficient of expansion containing as high as forty per cent nickel and a greater percentage of iron, and the part of higher coefficient of expansion consisting of metallic elements approximately in following percentage—

|              |       |                |
|--------------|-------|----------------|
| Carbon       | ----- | .25 to .35     |
| Silicon      | ----- | 1.75 to 2.00   |
| Chromium     | ----- | 13.25 to 14.00 |
| Nickel       | ----- | 7.25 to 7.75   |
| Copper       | ----- | 2.00 to 4.00   |
| Wrought iron | ----- | 72.50 to 71.90 |

3. A bimetallic thermostat comprising two metallic elements secured together and having marked difference in coefficients of expansion within a temperature range of approximately 200 degrees F., the said differences in coefficient of expansion producing a practically constant degree of movement per degree of change in temperature within the said range, both elements having a predominant iron content and the element of lower coefficient of expansion having as high as forty per cent of nickel and the element of higher coefficient of expansion having a nickel content of not more than eight per cent, and a chromium content of approximately fourteen per cent.

4. A heat responsive device comprising two members secured together throughout their length, one being a corrosion resistant iron alloy of chromium containing from 10 to 15% of chromium and the other member being an alloy of iron and nickel having a coefficient of expansion less than that of the first said member.

5. A thermostatic device comprising two members united together, each having dis-

similar thermal characteristics and each consisting of an alloy of iron in a predominating amount, one member containing approximately 36% of nickel and the other member from 10 to 15% chromium.

5 6. A thermostatic device comprising two members united together, one composed of invar and the other of a high resistance iron alloy containing approximately 18% of chromium.

10 In testimony whereof, I sign this specification.

WILLIAM M. CHACE.

15

20

25

30

35

40

45

50

55

60

65